

1

2,777,186

## PROCESS FOR THE PRODUCTION OF PERMANENT LOCALLY GOFFERED EFFECTS AND PRODUCTS THEREFROM

Fritz Vonaesch, Wattwil, Switzerland, assignor to Heberlein Patent Corporation, New York, N. Y., a corporation of New York

No Drawing. Application December 21, 1953,  
Serial No. 399,601

10 Claims. (Cl. 26—69)

This invention relates to the production of permanent locally goffered effects, especially on cotton fabrics; and to products obtained thereby. It is known to produce permanent locally goffered effects on fabrics by means of thermosetting synthetic resins by printing the fabric prior to the goffering with a synthetic resin precondensate according to a predetermined pattern. Thereupon, the fabric was dried, subjected to all-over goffering and then the synthetic resin precondensate was hardened in the pattern by heating to an elevated temperature. Finally, the fabric was washed and dried whereby the goffered effect on the parts not treated with the synthetic resin was removed by the washing process. Alternatively the effect was produced by impregnating the fabric with a synthetic resin precondensate and inhibiting resin condensation on the desired parts, for instance by printing same with an alkaline agent.

It also has been proposed to remove the goffered effects from the unprinted portions of fabrics by alkali of shrinkage strength as well as to parchmentize the unprinted portions with sulphuric acid. All of the prior processes, however, either result in leaving evidences of the goffering in portions intended to be free of goffering, or injuring the printed goffered portions and otherwise changing the appearance and character of the fabric.

The principal object of the present invention is accordingly to produce a simple, efficient process for producing such effects and to overcome the difficulties mentioned.

The invention accordingly consists of the novel products as well as the novel processes and steps of processes according to which such products are manufactured, the specific embodiments of which are described hereinafter by way of example and in accordance with which I now prefer to practice the invention.

I have found in accordance with my invention that the permanent locally goffered effects can be satisfactorily produced by printing a local pattern on a cotton fabric with a formaldehyde resin precondensate. The fabric so printed with the precondensate is over-all goffered and the fabric so printed is condensed so that the resin is thermoset. The fabric so treated is washed to remove some of the goffer from the unprinted portions and is then treated with a goffer-removing agent. This goffer-removing agent removes the remaining goffer in the unprinted portions without affecting the appearance of the fabric. The agents employed are discussed more fully below.

I have found in accordance with my invention that, upon printing a local pattern on a cotton fabric with a formaldehyde resin precondensate and over-all goffering the printed fabric and condensing the printed pattern, it is possible to remove the goffer from the unprinted portions without changing the appearance of the fabric unprinted with the resin. I have ascertained that some of this goffering effect can be removed by treatment by washing with water, but even if I add soap to this water and apply it at high temperatures, say up to 70° C., there still remains in the portions untreated with the resin remnants of the goffering. For a practical process it is important

2

that these remnants be removed. It is known that all of the goffering can be taken out by the use of caustic soda of mercerizing strength, that is about 28°—38° Bé., but the difficulty with such treatment is that it definitely alters the appearance of the fabric. Thus, if it is done without tension, the fabric crinkles. If it is done with tension, the tension applied is such that the goffered effect in the resin-printed portions is damaged by pulling out of shape. On the other hand it is known that all of the goffering can be taken out of the unprinted portions by treatment with a parchmentizing agent such as sulphuric acid, but the result of treatment with this parchmentizing agent is that the fabric becomes transparent and stiffened in the unprinted portions. In addition resins such as are used here are readily attacked by such parchmentizing acid and the printed portions are consequently damaged.

I have found, however, in accordance with my invention that, after condensation of the printed portions of the fabric and after washing with water to remove some of the goffering in the unprinted portion, I can remove the remainder of the goffering in the unprinted portion by treatment with a goffer-removing agent which not only will remove all traces of the goffered effect in the unprinted portions but will do this without damage to the goffered effect in the printed portions. Such agents include aqueous solutions of sodium hydroxide of 10—22° Bé. and aqueous solutions of potassium hydroxide of 10—25° Bé. These solutions may be employed at room temperatures and above. In addition other agents which may be employed are, but without limitation, solutions of zinc chloride and calcium thiocyanate which may be employed in concentrations up to saturation but are employed at room temperature. In other words, they are employed under conditions so that they do not parchmentize the fabric. I find it important to wash out the condensed fabric primarily for two reasons. One, the condensation is usually conducted with a catalyst and it is important that this catalyst be removed prior to treatment with the goffer-removing agent. Two, it is almost always the case that the goffering roll produces compressed portions in the fabric which the subsequent treatment with the goffer-removing agent described will have difficulty in removing. With the washing treatment with water these portions are softened up and no trace of them remains after the goffer-removing agent has acted.

As thermosetting synthetic resin precondensates in connection with the present process we use: condensates of formaldehyde and urea, thiourea, ethylene urea and homologues of same, urone, acetylene diurea, dicyandiamide, melamine, phenol and phenol derivatives; as well as suitable mixtures of these resin components. They are applied together with the usual acid or alkaline catalysts. Also ketone aldehyde precondensates may be used. Furthermore, also suitable solvent dyestuffs, pigments or compounds forming same, as well as metal powder, if desired, together with dyestuffs for the purpose of the production of gold, silver, and copper effects, can be added to the synthetic resin precondensate.

As fabrics, cotton fabrics, such as cotton percale, cotton cretonne or cotton print cloth are used. Fabrics pre-dyed in lighter shades and/or color printed can be provided locally with a resin compound containing a color pigment if desired. Besides the resin print, also a regular color print can be executed. If darker shades are desired besides light colored goffered effects, the fabric is preferably dyed afterwards.

The following are examples of the process as I now prefer to practice it. It is to be understood that these examples are illustrative of the process and the process is not to be considered as confined thereto except as indicated in the appended claims.

**3**  
*Examples*

1. A bleached cotton print fabric is printed in a predetermined pattern with the following printing compound:

|                                                                                                                | Grams |
|----------------------------------------------------------------------------------------------------------------|-------|
| Hexamethylol melamine-precondensate                                                                            | 175   |
| Water                                                                                                          | 200   |
| Concentrated ammonia conc. sp. gr. 0.91                                                                        | 5     |
| Tylose TWA, aqueous solution 65 gr./litre (methyl cellulose of Kalle & Co. A. G., Wiesbaden-Biebrich, Germany) | 500   |
| Ammonium thiocyanate-water, 1 part of thiocyanate by weight to 1 part of water                                 | 20    |
| Indanthrene scarlet GG, paste (Schultz Index, supplemental volume II, No. 1289a)                               | 100   |
|                                                                                                                | 1000  |

Then the goods are dried at about 40° C. and goffered all over at about 200° C., then washed for a short time and dried without tension. Thereupon, the goods are impregnated on a padding machine with aqueous sodium hydroxide of 20° Bé. at room temperature, kept for some time, at least 10 seconds up to about 5 minutes, in this condition, then dyed with hot and cold water, framed and finished in the usual manner. One gets a scarlet coloured goffered pattern on a smooth, white ground.

2. A cotton percale fabric, dyed light green, is printed in a pattern with the following printing compound:

|                                                                | Grams |
|----------------------------------------------------------------|-------|
| Hexamethylol melamine-precondensate                            | 200   |
| Water                                                          | 195   |
| Carro bean meal thickener 25:1000 (25 gr. meal/litre of water) | 540   |
| Ammonia conc.                                                  | 5     |
| Ammonium chloride-water, 1:1 by weight                         | 10    |
| Lampblack                                                      | 50    |
|                                                                | 1000  |

The printed goods are dried at about 40° C., goffered all over at 200° C., condensed at 140° C. for 4 minutes, washed and dried without tension. Thereupon, the goods are impregnated on a pad with aqueous potassium hydroxide of 20° Bé., at room temperature, kept in this condition for 15 minutes, then dyed with hot and cold water, framed and completed in the usual manner.

One gets a gray goffered design on light green, smooth background.

3. A bleached cotton cretonne is printed as indicated in Example 1, dried, goffered all over, condensed, washed and dried. Then, the goods are impregnated with an aqueous zinc chloride solution (about 600 gr. zinc chloride/litre), kept at room temperature for 2 minutes in this condition, then washed out and framed. Then the fabric is overdyed with a substantive blue dyestuff whereby the goffered parts are reserved. The fabric is finished in the usual way.

In this way one gets scarlet coloured goffered effects on a blue dyed ground.

4. A bleached cotton print cloth is printed in a multi-colour pattern. The printing compound for printing the ground is the same as in Example 1, which produces a print ready for permanent goffering. Instead of Indanthrene scarlet GG paste, the same amount of Indanthrene brilliant green 4G (Schultz Index No. 1269) is employed. For the remaining colours, regular vat print pastes are used. After the printing and drying at about 40° C., the goods are goffered all over at 180–200° C., then they are condensed at 140° C. for 4 minutes, steamed as usual for vat dyestuffs, oxidized, washed, soaped, scoured and dried without tension. Thereupon, the goods are treated as in Example 1 with aqueous sodium hydroxide and finished, whereby one gets a green goffered ground alongside a smooth colour print on a white ground.

**4**

5. A bleached cotton percale is printed in a five-colour pattern. Three of these colours, scarlet, pink and blue, are applied to produce a print ready for permanent goffering. For the scarlet colour, a printing compound is used according to Example 1; for the pink and blue colour, respectively, I use similar compositions to those of Example 1, using the same amounts of Indanthrene brilliant pink R paste (Schultz Index No. 1345) and Indanthrene blue GCD (Schultz Index No. 1234). For the remaining two colours regular Orema printing pastes of Ciba A. G. are used. These latter appear in the smooth non-goffered portions. The fabric, after printing, is dried and goffered as in the preceding example.

After the goods are finished according to Example 1, one gets a design with scarlet, pink and blue coloured permanent goffered parts alongside smooth parts printed in the other two colours.

6. A bleached cotton cretonne fabric is pattern-printed with the following printing compound:

|                                                                                                       | Grams |
|-------------------------------------------------------------------------------------------------------|-------|
| Beckamine P 468 (ketone-formaldehyde-precondensate of the Reichhold Chemical Inc., Detroit, U. S. A.) | 175   |
| Water                                                                                                 | 100   |
| Ahcowel G (fatty acid amide condensate of the Arnold Hoffman Co., Providence, Rhode Island, U. S. A.) | 30    |
| Carro bean meal thickener aqueous (25 gr. meal/litre of water)                                        | 500   |
| Indanthrene gold yellow RK (Schultz Index, supplemental volume II, No. 1286c)                         | 100   |
| Soda ash                                                                                              | 14    |
| Water                                                                                                 | 81    |
|                                                                                                       | 1000  |

After printing the goods are dried at about 40° C. and goffered at about 200° C. Thereupon they are condensed for 2 minutes at 150° C., then washed for a short time and dried without tension. Thereupon the goods are impregnated on a pad with a concentrated aqueous solution of calcium thiocyanate (about 700 gr./litre), kept for 5 minutes in this condition at room temperature, thoroughly washed and finished in the usual way.

One gets a yellow goffered pattern on a smooth, white ground.

The expression "mild goffer-removing agent" is intended to indicate solutions of caustic soda of 10–22° Bé. and of potash lye of 10–25° Bé. as well as aqueous solutions of zinc chloride and calcium thiocyanate and equivalent agents which are capable of removing the goffering without causing shrinkage or parchmentizing of cotton fabrics.

What I claim is:

1. A process for the production of permanent locally goffered effects on a fabric alongside smooth portions thereof which comprises, printing a local pattern on cotton fabric with a formaldehyde resin precondensate, overall goffering the printed fabric, condensing the printed pattern, washing the condensed fabric to remove some of the goffering from the unprinted portion, and then impregnating the goffered goods with a mild goffer-removing agent to remove the remaining goffer in the unprinted portions without otherwise affecting the appearance thereof.

2. A process according to claim 1, in which the goffer-removing agent is a solution of caustic soda of 10–22° Bé.

3. A process according to claim 1, in which the goffer-removing agent is a dilute solution of potash lye having a strength of 10–25° Bé.

4. A process in accordance with claim 1, in which the precondensate applied to the fabric for fixation of the goffered effects contains a coloring substance.

5. A process in accordance with claim 1, in which the synthetic resin is a methylol melamine.

6. A process in accordance with claim 1, in which the resin is a ketone aldehyde precondensate.

7. A cotton fabric treated in accordance with the process of claim 1.

8. A process for the production of permanent locally goffered effects on a fabric alongside smooth portions thereof which comprises, printing a local pattern on cotton fabric with a formaldehyde resin precondensate, overall goffering the printed fabric, condensing the printed pattern, washing the condensed fabric to remove some of the goffering from the unprinted portion, and then impregnating the goffered goods with an aqueous solution of zinc chloride at about room temperature to remove the remaining goffer in the unprinted portions without otherwise affecting the appearance thereof.

9. A process for the production of permanent locally goffered effects on a fabric alongside smooth portions thereof which comprises, printing a local pattern on cotton fabric with a formaldehyde resin precondensate, overall goffering the printed fabric, condensing the printed pattern, washing the condensed fabric to remove some of the goffering from the unprinted portion, and then impregnating the goffered goods with an aqueous solution of calcium thiocyanate at about room temperature

5

10

15

20

to remove the remaining goffer in the unprinted portions without otherwise affecting the appearance thereof.

10. A process for the production of permanent locally goffered effects on a fabric alongside smooth portions thereof which comprises, printing a local pattern on cotton fabric with a methylol melamine precondensate, over-all goffering the printed fabric, condensing the printed pattern, washing the condensed fabric to remove some of the goffering from the unprinted portion, and then impregnating the goffered goods with a solution of caustic soda 10-22° Bé. to remove the remaining goffer in the unprinted portions without otherwise affecting the appearance thereof.

**References Cited in the file of this patent**

**UNITED STATES PATENTS**

|           |                      |               |
|-----------|----------------------|---------------|
| 2,103,587 | Lantz et al. -----   | Dec. 28, 1937 |
| 2,161,223 | Bener -----          | June 6, 1939  |
| 2,520,699 | Sowerby et al. ----- | Aug. 29, 1950 |
| 2,622,994 | Lippert et al. ----- | Dec. 23, 1952 |

**FOREIGN PATENTS**

|         |                     |                |
|---------|---------------------|----------------|
| 592,649 | Great Britain ----- | Sept. 24, 1947 |
|---------|---------------------|----------------|